

# UNITED STATES PATENT OFFICE.

LUCY C. BOLTON, OF PEORIA, ILLINOIS.

## VARNISH FOR FINISHING WOOD.

SPECIFICATION forming part of Letters Patent No. 377,797, dated February 14, 1888.

Application filed October 12, 1887. Serial No. 252,156. (No specimens.)

*To all whom it may concern:*

Be it known that I, LUCY C. BOLTON, a citizen of the United States, residing at Peoria, in the county of Peoria and State of Illinois, 5 have invented certain new and useful Improvements in Varnishes; and I do hereby declare the following to be a full, clear, and exact description of the invention, such as will enable others skilled in the art to which it appertains 10 to make and use the same.

My invention relates to a compound for varnishing wood and other surfaces.

The object of my invention is to provide a compound or mixture which can be easily applied, and which will dry quickly and leave a 15 beautiful smooth surface resembling polished hard wood.

With these ends in view my invention consists in combining the following ingredients: 20 one pint of pure water, one table-spoonful of kerosene or other mineral oil, one ounce of common glue, one-quarter of an ounce of salt-peter, one-quarter of an ounce of alum, and one-half an ounce of tartaric acid. These ingredients are to be placed in a suitable receptacle 25 and mixed together until all are thoroughly assimilated, after which the compound will be ready for use. It can be applied to any smooth surface by means of a brush; but the way in 30 which I prefer to apply it is by rubbing it on with a cloth. After applying and before it becomes dry the operator can, by use of a piece of rubber, form any fanciful designs of grain-

ing with the greatest facility. Curly maple, walnut, and various other woods can be imitated with great success. 35

When dry, the compound gives to the wood or other material treated a highly-polished, smooth, and beautiful surface, and when applied to doors, furniture, &c., it gives them a 40 fine elegant finish, and adds greatly to their durability, as the composition will not rub off, and only becomes slightly worn after long usage.

Although in manufacturing my compound I 45 prefer to mix the various ingredients in the proportions before stated, yet I do not wish to limit myself strictly to said proportions, as it is evident that they can be slightly varied without materially changing the nature of the 50 resulting compound or departing from the spirit and scope of my invention.

Having thus fully described my invention, what I claim as new, and desire to secure by Letters Patent, is— 55

A varnish or finishing compound consisting of water, mineral oil, glue, salt-peter, alum, and tartaric acid mixed together, substantially as described.

In testimony whereof I affix my signature in 60 presence of two witnesses.

LUCY C. BOLTON.

Witnesses:

E. BURROUGHS,  
IRENE BURROUGHS.